

## UNITED STATES PATENT OFFICE

2,542,553

## MINERAL OIL COMPOSITION

Louis A. Mikeska and Paul V. Smith, Jr., Westfield, N. J., assignors to Standard Oil Development Company, a corporation of Delaware

No Drawing. Application December 2, 1948,  
Serial No. 63,188

6 Claims. (Cl. 252—46.6)

1

This invention pertains to extreme pressure lubricants and compositions for imparting extreme pressure or load carrying properties to lubricating oils. The invention also pertains to a method for preparing extreme pressure agents, incorporating elements such as sulfur, phosphorus, and the like, in such a manner that they will be available for suitable chemical activity under heavy load conditions.

As is well understood in the art, ordinary mineral base lubricating oils and greases which are used to lubricate opposed metal surfaces are likely to fail under extremely heavy load conditions. For example, certain machine elements such as the hypoid gears commonly used in automotive vehicles, may be subjected at times to extremely heavy pressures of the order of hundreds of thousands of pounds per square inch. If the film of lubricating oil separating the opposed elements fails, as it is likely to do under such pressure, the surfaces will contact each other directly, generating high temperatures due to friction, with resultant seizure or excessive wear and early failure. Extreme pressure additives containing active sulfur, phosphorus, or chlorine, or two or more of these, are effective to react immediately with the metal surfaces at their higher temperatures to form a protective metal sulfide, phosphide, or chloride film which serves temporarily as a lubricating medium until the normal oil film between the parts can be reestablished. Extreme pressure additives are, therefore, reactive with the metals they lubricate to form extremely thin protective films thereon when the temperature rises due to normal oil film failure.

It is known to the art (J. Inst. Petr., v. 31; 73 (1945) that the presence of a  $\text{Cl}_3\text{C}$ —group in a compound tends to impart extreme pressure properties thereto. For example, condensation products of chloral with mercaptans such as ethyl, n-butyl, isobutyl, phenol, benzyl, thioglycollic acid, thiosalicylic acid and mixed petroleum mercaptans in the boiling range 20° to 50° C. are good extreme pressure additives.

It has now been found that compositions having extreme pressure properties and other desirable properties for use in lubricating oil compositions and the like may be prepared by treating chloral or its hydrate with a mercaptan to form the hemi-mercaptal of chloral which itself is an excellent oiliness and extreme pressure agent. The fur-

2

ther reaction of chloral hemi-mercaptals with phosphorus pentasulfide or phosphorus sesquisulfide gives products which impart exceptional oiliness and extreme pressure properties to mineral oil blends. Equally effective products can be obtained by converting the hemi-mercaptals to alkali xanthates which are in turn condensed with sulfur di- or monochloride to yield the correspond polysulfides.

10 The hemi-mercaptals are prepared simply by treating chloral or its hydrate with the desired mercaptan. Mercaptans containing from 2 to 20 carbon atoms may be used. However, mercaptans having from 8 to 20 carbon atoms are preferred.

Simple hemi-mercaptals of chloral are reacted with phosphorous pentasulfide by refluxing the reactants in the presence of some solvent such as dioxane, toluene, etc. By reacting simple hemi-20 mercaptals first with carbon disulfide and an alkali, a xanthate may be formed which, by reaction with sulfur dichloride, forms the desired xanthogen trisulfide.  $\text{S}_2\text{Cl}_2$ ,  $\text{SOCl}_2$ , or  $\text{ClSCl}_2$  may be used in place of sulfur dichloride.

25 Generally, the products of this invention may be represented by the generalized formula,



wherein R represents an alkyl group, X represents H in the case of simple hemi-mercaptals and



in the case of xanthogen trisulfide, Y represents sulfur or oxygen, and n represents the integer 1 or 2.

40 The reaction product of hemi-mercaptals and phosphorus pentasulfide contains very little phosphorus. One sample analysis shows as little as 0.04%. The reaction is complex and the structure of the product has not been fully determined. Analysis of a sample indicated the following weight percentages:

|            | Per cent |
|------------|----------|
| Phosphorus | 0.044    |
| Sulfur     | 17.88    |
| Chlorine   | 25.86    |

## 3

In producing the additives of the present invention, chloral hydrate is simply heated together with a suitable mercaptan. A solvent such as dioxane may be used if desired. The reaction time may vary from 0.25 to 3 hours. The hemi-mercaptopal thus formed may be used as such or it may be further reacted with  $P_2S_5$  by simply refluxing the entire mixture for 3 hours. The xanthogen trisulfide is formed by reacting the chloral hemi-mercaptopal with sodium or 10 potassium hydroxide and an excess of carbon disulfide. The metal xanthate thus formed is then reacted with sulfur dichloride by refluxing in the presence of a solvent such as benzene.

It will be understood that compositions of the types referred to in the present application may be added in various quantities to various types of oils as will be obvious to those skilled in the art. They may be added to relatively light oils, such as oils of automotive engine grades, for the purpose of increasing oxidation stability although normally they will be used more widely in heavier oils, such as SAE 80, 90, or 140 grade for the lubrication of hypoid gears or other machine elements encountering extreme pressure conditions. They may also be used in cutting oils, in soluble cutting oils in conjunction with sodium sulfonates and with other appropriate emulsifying agents. For use in gear oils, proportions of 5% to 20% by weight of the additives are preferred, 10% being a common useful proportion. It will be understood, however, that proportions as low as about 1% may be employed. For concentrates, to be added to oils by the consumer according to his needs, the additive products of this invention may be marketed straight or in 10% to 80% solutions in mineral oil of appropriate grade. The mineral lubricating oils having viscosities between about 35 S. S. U. and 1,000 S. S. U. at 210° F. are preferred.

Various conventional additives may be employed in connection with the extreme pressure compounds described above, such as thickeners, oiliness agents, oxidation inhibitors, tackiness agents, viscosity index improvers, pour point depressants, and the like. These materials may also be used in greases thickened with soaps, carbon blacks, silica gels and other known grease-forming materials.

The invention will be more fully understood by reference to the following examples:

## Example I

A sample of tertiary-octyl hemi-mercaptopal of chloral, a sample of tertiary-dodecyl hemi-mercaptopal of chloral and a sample of tertiary-hexadecyl hemi-mercaptopal of chloral were prepared by heating together dioxane, chloral hydrate, and tertiary-octyl mercaptan, tertiary-dodecyl mercaptan, and tertiary-hexadecyl mercaptan respectively at the reflux temperature of the mixture for a period ranging from 0.25 to 3 hours. The resulting compound was tested on the Almen machine using the procedure described in the patent to J. O. Almen, U. S. 2,001,861, with the following results:

|                                                | Gradual | Shock |
|------------------------------------------------|---------|-------|
| Tertiary-octyl hemi-mercaptopal of chloral     | 15      | 15    |
| Tertiary-dodecyl hemi-mercaptopal of chloral   | 15      | 13    |
| Tertiary-hexadecyl hemi-mercaptopal of chloral | 15      | 11    |

## Example II

Samples of tertiary-octyl, tertiary-dodecyl and

## 4

tertiary-hexadecyl hemi-mercaptopal of chloral, prepared in accordance to the procedure of Example I, were treated with phosphorus pentasulfide. The reaction products were tested in the Almen machine with the following results:

|                                                             | Gradual | Shock |
|-------------------------------------------------------------|---------|-------|
| Product from Tertiary-octyl hemi-mercaptopal of chloral     | 15      | 15    |
| Product from Tertiary-dodecyl hemi-mercaptopal of chloral   | 15      | 15    |
| Product from Tertiary-hexadecyl hemi-mercaptopal of chloral | 15      | 11-12 |

## Example III

Samples of tertiary-octyl, tertiary-dodecyl, and tertiary-hexadecyl hemi-mercaptopal of chloral, prepared in accordance with the procedure of Example I, were treated with  $CS_2$  and  $NaOH$  to form the sodium xanthates. These xanthates were further reacted with  $SCl_2$  to form the corresponding xanthogen trisulfides. The reaction products were tested in the Almen machine with the following results:

|                                                             | Gradual | Shock |
|-------------------------------------------------------------|---------|-------|
| Product from Tertiary-octyl hemi-mercaptopal of chloral     | 15      | 15    |
| Product from Tertiary-dodecyl hemi-mercaptopal of chloral   | 15      | 13-14 |
| Product from Tertiary-hexadecyl hemi-mercaptopal of chloral | 15      | 9-10  |

What is claimed is:

1. A composition consisting essentially of a mineral oil base stock containing 1% to 20% by weight based on total composition, of a compound having the formula



wherein R represents an alkyl group containing from 2 to 20 carbon atoms, and Y represents an element selected from the class consisting of oxygen and sulfur.

2. A composition consisting essentially of a mineral oil base stock containing from 1% to 20% by weight based on a total composition, of a compound having the formula



wherein R represents an alkyl group containing 2 to 20 carbon atoms.

3. A composition consisting essentially of a mineral oil base stock containing from 1% to 20% by weight, based on total composition, of a compound having the formula



wherein R represents an alkyl group containing from 2 to 20 carbon atoms.

4. A composition consisting essentially of a mineral oil base stock containing from 1% to 20% by weight, based on total composition, of a compound having the formula



5. A composition consisting essentially of a mineral oil base stock containing from 1% to 20% by weight, based on total composition, of a compound having the formula



6. A composition consisting essentially of a mineral oil base stock containing 1% to 20% by 10 weight based on the total composition, of a compound having the formula



LOUIS A. MIKESKA.  
PAUL V. SMITH, JR.

## REFERENCES CITED

The following references are of record in the file of this patent:

## UNITED STATES PATENTS

| Number    | Name          | Date           |
|-----------|---------------|----------------|
| 2,228,252 | Berger et al. | Jan. 14, 1941  |
| 2,247,045 | Berger et al. | June 24, 1941  |
| 2,329,324 | Berger et al. | Sept. 14, 1943 |

## OTHER REFERENCES

15 Pages 527-530 of the Journal of the Institute of Petroleum, vol. 33, 1947. Article by Davey entitled "Some Extreme Pressure Lubricating Oil Additives."